



US009235148B2

(12) **United States Patent**  
**Sugahara et al.**

(10) **Patent No.:** **US 9,235,148 B2**  
(b4) **Date of Patent:** **Jan. 12, 2016**

(54) **ELECTROSTATIC LATENT IMAGE  
DEVELOPING TONER**

(71) **Applicant:** **KYOCERA DOCUMENT  
SOLUTIONS INC.**, Osaka (JP)

(72) **Inventors:** **Masanori Sugahara**, Osaka (JP);  
**Toshiki Takemori**, Osaka (JP)

(73) **Assignee:** **KYOCERA Document Solutions Inc.**,  
Osaka (JP)

(\*) **Notice:** Subject to any disclaimer, the term of this  
patent is extended or adjusted under 35  
U.S.C. 154(b) by 41 days.

(21) **Appl. No.:** **14/085,415**

(22) **Filed:** **Nov. 20, 2013**

(65) **Prior Publication Data**

US 2014/0141368 A1 May 22, 2014

(30) **Foreign Application Priority Data**

Nov. 22, 2012 (JP) ..... 2012-256836

(51) **Int. Cl.**  
**G03G 9/087** (2006.01)  
**G03G 9/08** (2006.01)

(52) **U.S. Cl.**  
CPC ..... **G03G 9/0821** (2013.01); **G03G 9/08782**  
(2013.01); **G03G 9/08795** (2013.01); **G03G  
9/08797** (2013.01)

(58) **Field of Classification Search**  
CPC ..... G03G 9/0821; G03G 9/08782; G03G  
9/08795; G03G 9/08797

USPC ..... 430/108.4  
See application file for complete search history.

(56) **References Cited**

U.S. PATENT DOCUMENTS

|                  |         |                                 |
|------------------|---------|---------------------------------|
| 5,635,325 A      | 6/1997  | Inaba et al.                    |
| 7,056,638 B1     | 6/2006  | Tomita et al.                   |
| 2002/0172879 A1  | 11/2002 | Kada et al.                     |
| 2007/0111128 A1* | 5/2007  | Patel et al. .... 430/108.4     |
| 2010/0028795 A1  | 2/2010  | Magome et al.                   |
| 2013/0071783 A1* | 3/2013  | Kuroyama .... 430/108.4         |
| 2013/0164669 A1* | 6/2013  | Yamashita et al. .... 430/108.4 |

FOREIGN PATENT DOCUMENTS

|    |               |        |
|----|---------------|--------|
| EP | 1223474 A2    | 7/2002 |
| EP | 2287673 A1    | 2/2011 |
| JP | H08-50368 A   | 2/1996 |
| JP | 2000-267338 A | 9/2000 |

(Continued)

OTHER PUBLICATIONS

The extended European search report issued on Feb. 21, 2014, which corresponds to European Patent Application No. 13193799.7-1303 and is related to U.S. Appl. No. 14/085,415.

*Primary Examiner* — Christopher Rodee

(74) **Attorney, Agent, or Firm:** Studebaker & Brackett PC

(57) **ABSTRACT**

Electrostatic latent image developing toner includes at least a binder resin and a releasing agent. In the electrostatic latent image developing toner, a maximum thermal expansion coefficient difference ( $Sw_{max} - Sr_{max}$ ), which is a difference between a maximum value ( $Sw_{max}$ ) of a thermal expansion coefficient of the releasing agent and a maximum value ( $Sr_{max}$ ) of a thermal expansion coefficient of the binder resin, is 1 or more, and a temperature at which the thermal expansion coefficient of the releasing agent reaches a maximum is 60° C. or more to 75° C. or less.

**4 Claims, 3 Drawing Sheets**



(56)

**References Cited**

FOREIGN PATENT DOCUMENTS

JP 2002-006541 A 1/2002

JP 2007-114804 A 5/2007  
JP 2011-138120 A 7/2011  
WO WO 2012/029611 A1 \* 3/2012

\* cited by examiner



FIG. 1



FIG. 2



FIG. 3



FIG. 4



FIG. 5



FIG. 6

# ELECTROSTATIC LATENT IMAGE DEVELOPING TONER

## INCORPORATION BY REFERENCE

The present application claims priority under 35 U.S.C. §119 to Japanese Patent Application No. 2012-256836, filed Nov. 22, 2012. The contents of this application are incorporated herein by reference in their entirety.

## BACKGROUND

The present application relates to electrostatic latent image developing toner.

Regarding toner used for electrophotography, a toner having excellent low temperature fixability is desired for achieving energy saving, compactness in device size, or the like. The toner having excellent low temperature fixability can be fixed by heating a fixing roller to a minimum. However, in many cases, the toner having excellent low temperature fixability includes a binder resin having a low melting point and a low glass transition point, and a releasing agent having a low melting point. Therefore, generally, the toner having excellent low temperature fixability has a problem of being likely to aggregate when stored at high temperature or to cause high temperature offset caused by the toner which sticks by melting to the heated fixing roller.

To solve the problem as described above, the toner with at least resin and wax is suggested. The resin included in this toner is a condensed resin. Then, the wax is included in each toner particle and is localized in the vicinity of a surface of the toner particles.

## SUMMARY

Specifically, the present application provides the following.

An electrostatic latent image developing toner according to the present disclosure includes at least a binder resin and a releasing agent. A maximum thermal expansion coefficient difference ( $S_{w_{max}} - S_{r_{max}}$ ) is 1 or more, the maximum thermal expansion coefficient being a difference between a maximum value ( $S_{w_{max}}$ ) of a thermal expansion coefficient of the releasing agent and a maximum value ( $S_{r_{max}}$ ) of a thermal expansion coefficient of the binder resin that are measured by the thermomechanical analysis (TMA). A temperature at which the thermal expansion coefficient of the releasing agent reaches a maximum is 60°C. or more and 75°C. or less.

#### BRIEF DESCRIPTION OF THE DRAWINGS

FIG. 1 is a diagram showing thermal expansion coefficient curves of a releasing agent and a binder resin that are included in toner in Example 1.

FIG. 2 is a diagram showing thermal expansion coefficient curves of a releasing agent and a binder resin that are included in toner in Example 2.

FIG. 3 is a diagram showing thermal expansion coefficient curves of a releasing agent and a binder resin that are included in toner in Comparative Example 1.

FIG. 4 is a diagram showing thermal expansion coefficient curves of a releasing agent and a binder resin that are included in toner in Comparative Example 2.

FIG. 5 is a diagram showing thermal expansion coefficient curves of a releasing agent and a binder resin that are included in toner in Comparative Example 3.

1

2

FIG. 6 is a diagram showing thermal expansion coefficient curves of a releasing agent and a binder resin that are included in toner in Comparative Example 4.

## DETAILED DESCRIPTION

The following describes embodiments of the present disclosure in detail. The present disclosure is not limited to the embodiments below in any case, and is executable with modifications where appropriate within the scope of the present disclosure. It should be noted that for the point where descriptions are overlapped, the description may be omitted where appropriate, which, however, is not to limit the content of the present disclosure.

15 The electrostatic latent image developing toner according to the present disclosure (hereinafter, also referred to as the toner) includes at least a binder resin and a releasing agent. In addition, a maximum value of a thermal expansion coefficient of the releasing agent and a maximum value of a thermal 20 expansion coefficient of the binder resin, which are measured using thermomechanical analysis, have a predetermined relationship. Then, a temperature at which the thermal expansion coefficient of the releasing agent reaches a maximum is within a predetermined range.

25 The toner according to the present disclosure may include an optional component such as a colorant, a charge control agent, and magnetic powder other than the binder resin and the releasing agent. In addition, in the toner according to the present disclosure, an external additive may be added to a 30 surface of each toner base particle as necessary. In addition, the toner according to the present disclosure may also be mixed with a desired carrier and used as a two component developer. Hereinafter, regarding the toner according to the present disclosure, the following describes: essential components (binder resin and releasing agent) and optional components (colorant, charge control agent, magnetic powder, and external additive). Furthermore, the following describes, in order, a method of manufacturing the toner according to the present disclosure, a carrier that is used in the case of using the 35 40 toner according to the present disclosure as a two component developer, and the thermomechanical analysis (TMA). [Binder Resin]

[Binder Resin] Binder resin included in the toner is selected such that the maximum value of the thermal expansion coefficient of the releasing agent and the maximum value of the thermal expansion coefficient of the binder resin have a predetermined relationship. It should be noted that the maximum value of the thermal expansion coefficient is measured by thermomechanical analysis (TMA) that is to be described later. A specific example of the binder resin is a thermoplastic resin such as: styrene-based resin, acrylic resin, styrene-acrylic resin, polyethylene-based resin, polypropylene-based resin, vinyl chloride-based resin, polyester resin, polyamide resin, polyurethane resin, polyvinyl alcohol-based resin, vinyl ether-based resin, N-vinyl-based resin, or styrene-butadiene based resin. Among these resins, due to excellence in colorant dispersibility in the toner, toner chargeability, and toner fixability onto paper, the styrene-acrylic resin or the polyester resin is preferable. The following describes the styrene-acrylic resin and the polyester resin.

The styrene-acrylic resin is a copolymer of a styrene-based monomer and an acrylic monomer. For specific examples of the styrene-based monomer, it is possible to give a monomer such as: styrene,  $\alpha$ -methylstyrene, vinyltoluene,  $\alpha$ -chlorostyrene,  $\alpha$ -chlorostyrene, m-chlorostyrene, p-chlorostyrene, or p-ethylstyrene. For specific examples of the acrylic monomer, it is possible to give a monomer such as: (meth)acrylate

alkyl ester such as methyl acrylate, ethyl acrylate, n-propyl acrylate, iso-propyl acrylate, n-butyl acrylate, iso-butyl acrylate, 2-ethylhexyl acrylate, methyl methacrylate, ethyl methacrylate, n-butyl methacrylate, or iso-butyl methacrylate.

For the polyester resin, it is possible to use resin obtained by condensation polymerization of an alcohol component that is divalent or of a valence of 3 or more, and a carboxylic acid component that is divalent or of a valence of 3 or more, or by copolycondensation of these. For a component used for synthesizing the polyester resin, an alcohol component that is divalent or of a valence of 3 or more, or a carboxylic acid component that is divalent or of a valence of 3 or more can be used as below.

For specific examples of the alcohol component that is divalent or of a valence of 3 or more, it is possible to give: diols such as ethylene glycol, diethylene glycol, triethylene glycol, 1,2-propylene glycol, 1,3-propylene glycol, 1,4-butanediol, neopentyl glycol, 1,4-butenediol, 1,5-pentanediol, 1,6-hexanediol, 1,4-cyclohexanediethanol, dipropylene glycol, polyethylene glycol, polypropylene glycol, or poly-tetramethylene glycol; bisphenols such as bisphenol A, hydrogenated bisphenol A, polyoxyethylene-modified bisphenol A, or polyoxypropylene-modified bisphenol A; or alcohols having a valence of 3 or more such as sorbitol, 1,2,3,6-hexanetriol, 1,4-sorbitan, pentaerythritol, dipentaerythritol, tripentaerythritol, 1,2,4-butanetriol, 1,2,5-pentanetriol, glycerol, diglycerol, 2-methylpropanetriol, 2-methyl-1,2,4-butanetriol, trimethylolethane, trimethylolpropane, or 1,3,5-trihydroxymethylbenzene.

For specific examples of the carboxylic acid that is divalent or of a valence of 3 or more, it is possible to give: divalent carboxylic acid such as maleic acid, fumaric acid, citraconic acid, itaconic acid, glutaconic acid, phthalic acid, isophthalic acid, terephthalic acid, cyclohexanedicarboxylic acid, succinic acid, alkylsuccinic acid or alkenylsuccinic acid with n-butylsuccinic acid, n-butenylsuccinic acid, isobutylsuccinic acid, isobutenylsuccinic acid, n-octylsuccinic acid, n-octenylsuccinic acid, n-dodecylsuccinic acid, n-dodecylsuccinic acid, isododecylsuccinic acid, or isododecylsuccinic acid, adipic acid, sebatic acid, azelaic acid, and malonic acid; and carboxylic acid having a valence of 3 or more such as 1,2,4-benzene tricarboxylic acid (trimellitic acid), 1,2,5-benzene tricarboxylic acid, 2,5,7-naphthalenetetracarboxylic acid, 1,2,4-naphthalenetetracarboxylic acid, 1,2,4-butanetricarboxylic acid, 1,2,5-hexanetricarboxylic acid, 1,3-dicarboxyl-2-methyl-2-methylenecarboxypropane, 1,2,4-cyclohexanetricarboxylic acid, tetra(methylenecarboxyl)methane, 1,2,7,8-octanetetracarboxylic acid, pyromellitic acid, or EMPOL trimer acid. These carboxylic acid components that are divalent or of a valence of 3 or more may be formed as an ester-forming derivative such as acid halide, anhydride, or lower alkyl ester for use. Here, the "lower alkyl" refers to an alkyl group having the number of carbon atoms from 1 to 6.

In the case of using the polyester resin for the binder resin, a softening point of the polyester resin should preferably be 80°C. or more and 150°C. or less, and more preferably be 90°C. or more and 140°C. or less.

For the binder resin, for sufficient fixability, it is preferable to use a thermoplastic resin. However, not only can the thermoplastic resin be used by itself, but a crosslinking agent or a thermosetting resin can also be added to the thermoplastic resin. By partially introducing a crosslinking structure into the binder resin, it is possible to increase preservation stability, shape retention characteristic, and durability of the toner without reducing the toner fixability.

For the thermosetting resin that can be used with the thermoplastic resin, an epoxy resin or a cyanate-based resin is

preferable. Specific example of a preferred thermosetting resin includes a thermosetting resin such as: bisphenol A type epoxy resin, hydrogenated bisphenol A type epoxy resin, novolac-type epoxy resin, poly(alkylene ether)-type epoxy resin, cyclic aliphatic-type epoxy resin, or cyanate resin. Two or more types of these thermosetting resins can be used in combination with each other.

The glass transition point (Tg) of the binder resin should preferably be 50°C. or more and 65°C. or less, and more preferably be 50°C. or more and 60°C. or less. If the glass transition point (Tg) of the binder resin is too low, there is a case where the toner melts and clings together in a development section of an image forming apparatus, or part of the toner melts and clings together during the transportation of the toner container or during storage in the warehouse. On the other hand, if the glass transition point (Tg) of the binder resin is too high, the strength of the binder resin decreases, and it becomes more likely to increase toner attachment to a latent image bearing member. In addition, if the glass transition point (Tg) of the binder resin is too high, there is a tendency that the toner is not sufficiently fixed at low temperature.

It should be noted that the glass transition point (Tg) of the binder resin can be obtained from a change point of specific heat of the binder resin, using a differential scanning calorimeter (DSC). More specifically, it is possible to obtain the glass transition point (Tg) of the binder resin by measuring an endothermic curve of the binder resin, using, for example, DSC-6200 manufactured by Seiko Instruments Inc as a measurement device. By placing 10 mg of the binder resin in an aluminum pan as a measurement sample and using an empty aluminum pan as a reference, measurement is performed under conditions that: a measurement temperature range is 25°C. or more and 200°C. or less and a temperature increase rate is 10°C./min under normal temperature and normal humidity, so as to obtain the endothermic curve. Using the endothermic curve of the binder resin that is obtained, it is possible to obtain the glass transition point (Tg) of the binder resin.

It is preferable that the number average molecular weight (Mn) of the binder resin be 3000 or more and 6000 or less. In addition, it is preferable that the mass average molecular weight (Mw) of the binder resin be 200000 or more and 500000 or less. By setting the number average molecular weight (Mn) and the mass average molecular weight (Mw) of the binder resin within such a range, it is possible to obtain the toner that allows realizing sufficient fixability within a wider range of temperature. In addition, it is preferable that a molecular weight distribution (Mw/Mn), which is represented by a ratio between the number average molecular weight (Mn) and the mass average molecular weight (Mw), be 67 or more and 83 or less. By setting the molecular weight distribution of the binder resin within such a range, it is possible to obtain the toner that allows realizing sufficient fixability within a wider range of temperature. The number average molecular weight (Mn) and the mass average molecular weight (Mw) of the binder resin can be measured using, for example, a gel permeation chromatography.

[Releasing Agent]

The electrostatic latent image developing toner according to the present disclosure includes a releasing agent for improvements in fixability and offset resistance. The releasing agent is selected such that the maximum value of thermal expansion coefficient of the releasing agent and the maximum value of thermal expansion coefficient of the binder resin have a predetermined relationship and that the temperature at which the thermal expansion coefficient of the releasing agent reaches the maximum is within a predetermined range. It

should be noted that the maximum value of the thermal expansion coefficient of the releasing agent is measured using thermomechanical analysis (TMA) to be described later.

For the releasing agent, wax is preferable, and examples of the wax include: ester wax, polyethylene wax, polypropylene wax, fluororesin wax, Fischer-Tropsch wax, paraffin wax, or montan wax. For the ester wax, synthetic ester wax, or natural ester wax such as carnauba wax or rice wax can be given. Two or more types of these releasing agents can be used in combination with each other. Among these releasing agents, ester wax is more preferable.

Among the ester waxes, synthetic ester wax is preferable for reasons that appropriate selection of a synthetic material facilitates adjusting the maximum value of the thermal expansion coefficient of the releasing agent and the temperature at which the thermal expansion coefficient of the releasing agent reaches the maximum, and that such synthetic material is less likely to be affected by impurity.

A method for manufacturing the synthetic ester wax is not particularly limited as long as a chemical synthesis method is used. For example, the synthetic ester wax can be synthesized using a publicly known method such as a reaction between alcohol and carboxylic acid in the presence of an acid catalyst or a reaction between carboxylic acid halide and alcohol. It should be noted that the material for the synthetic ester wax may be derived from a natural material, for example, long-chain fatty acid manufactured from natural fat. In addition, for the synthetic ester wax, a commercially-available synthetic may be used.

For the releasing agent used for the toner according to the present disclosure, the thermal expansion coefficient of the releasing agent reaches the maximum at a temperature of 60° C. or more and 75° C. or less. By setting the temperature at which the thermal expansion coefficient of the releasing agent reaches the maximum within such a range, it becomes easier to obtain the toner having excellent high temperature offset resistance and excellent heat-resisting preservation stability.

If the temperature at which the thermal expansion coefficient of the releasing agent reaches the maximum is too low, an expansion of the releasing agent occurs in a low temperature range. Therefore, the toner, which includes the releasing agent of which the thermal expansion coefficient reaches the maximum at a temperature below 60° C., shows sufficient mold releasability in the low temperature range. However, such toner has poor releasability in a high temperature range. Thus, in the case of forming an image using the toner with a releasing agent of which the thermal expansion coefficient reaches the maximum at a temperature below 60° C., offset is more likely to occur at high temperature. In addition, when stored at high temperature, the toner, which includes the releasing agent of which the thermal expansion coefficient reaches the maximum at a temperature below 60° C., has poor preservation stability because the releasing agent is likely to exude from the toner.

On the other hand, if the temperature at which the thermal expansion coefficient of the releasing agent reaches the maximum is too high, the expansion of the releasing agent occurs in the high temperature range. Therefore, the toner, which includes a releasing agent of which the thermal expansion coefficient reaches the maximum at a temperature over 75° C., shows sufficient mold releasability in the high temperature range. However, such toner has difficulty in performing sufficient mold releasability within the low temperature range, and therefore has poor low temperature fixability.

The average carbon number of the releasing agent should preferably be 38 or more and 42 or less, and more preferably be 39 or more and 41 or less. By setting the average carbon

number of the releasing agent within such a range, it becomes easier to obtain the toner having excellent high temperature offset resistance and heat-resisting preservation stability. In addition, by setting the average carbon number of the releasing agent within such a range, it becomes easier to adjust the temperature at which the thermal expansion coefficient of the releasing agent reaches the maximum, which is measured using thermomechanical analysis (TMA), to 60° C. or more and 75° C. or less. For example, it is possible to decrease the temperature at which the thermal expansion coefficient of the releasing agent reaches the maximum by reducing the average carbon number of the releasing agent. In addition, it is possible to increase the temperature at which the thermal expansion coefficient of the releasing agent reaches the maximum by increasing the average carbon number of the releasing agent.

The amount of use of the releasing agent should preferably be 1 part by mass or more and 5 parts by mass or less, with respect to 100 parts by mass of the binder resin. If the amount of use of the releasing agent is too small, there is a case where a desired effect cannot be produced in suppressing occurrence of offset or image smearing. On the other hand, if the amount of use of the releasing agent is too large, there is a case where the preservation stability of the toner decreases due to the toner melted and clinging together.

[Colorant]

The electrostatic latent image developing toner according to the present disclosure may include a colorant in the binder resin. The colorant included in the toner is appropriately selected from among publicly known pigments or dyes according to the color of toner particles. For specific examples of the preferred colorant to be added to the toner, it is possible to give: a black pigment such as carbon black, acetylene black, lampblack, or aniline black; a yellow pigment such as chrome yellow, zinc yellow, cadmium yellow, yellow iron oxides, mineral fast yellow, nickel titanium yellow, Naples yellow, naphthol yellow S, hansa yellow G, hansa yellow 10G, benzidine yellow G, benzidine yellow GR, quinoline yellow lake, permanent yellow NCG, or tartrazine lake; an orange pigment such as orange chrome, molybdenum orange, permanent orange GTR, pyrazolone orange, vulcan orange, or indanthrene brilliant orange GK; a red pigment such as red iron oxide, cadmium red, red lead, cadmium mercury sulfide, permanent red 4R, lithol red, pyrazolone red, watching red calcium salt, lake red D, brilliant carmin 6B, eosin lake, rhodamine lake B, alizarin lake, or brilliant carmin 3B; a purple pigment such as manganese violet, fast violet B, or methyl violet lake; a blue pigment such as Prussian blue, cobalt blue, alkali blue lake, Victoria blue partial chlorinated product, fast sky blue, or indanthrene blue BC; a green pigment such as chrome green, chromium oxide, pigment green B, malachite green lake, or final yellow green G; a white pigment such as zinc oxide, titanium oxide, antimony white, or zinc sulfide; and an extender pigment such as baryta powder, barium carbonate, clay, silica, white carbon, talc, or alumina white. Two or more types of these colorants can be used in combination with each other for the purpose of adjusting a hue of the toner to a desired hue.

The amount of use of the colorant should preferably be 1 part by mass or more and 10 parts by mass or less, with respect to 100 parts by mass of the binder resin, and more preferably be 3 parts by mass or more and 8 parts by mass or less.

[Charge Control Agent]

The electrostatic latent image developing toner according to the present disclosure may include a charge control agent as necessary. The charge control agent is used for obtaining the toner having excellent durability and stability through

improvements in a charge level stability and a charge rise characteristic of the toner, which indicates whether or not charging the toner up to a predetermined charge level is possible within the short time. In the case of positively charging the toner for performing development, a positively chargeable charge control agent is used. On the other hand, in the case of negatively charging the toner for performing development, a negatively chargeable charge control agent is used.

The type of the charge control agent can be appropriately selected from among charge control agents used for toner since before. For specific examples of the positively chargeable charge control agent, it is possible to give: an azine compound such as pyridazine, pyrimidine, pyrazine, ortho-oxazine, meta-oxazine, para-oxazine, ortho-thiazine, meta-thiazine, para-thiazine, 1,2,3-triazine, 1,2,4-triazine, 1,3,5-triazine, 1,2,4-oxadiazine, 1,3,4-oxadiazine, 1,2,6-oxadiazine, 1,3,4-thiadiazine, 1,3,5-thiadiazine, 1,2,3,4-tetrazine, 1,2,4,5-tetrazine, 1,2,3,5-tetrazine, 1,2,4,6-oxatriazine, 1,3,4,5-oxatriazine, phthalazine, quinazoline, or quinoxaline; direct dyes made of an azine compound such as azine fast red FC, azine fast red 12BK, azine violet BO, azine brown 3G, azine light brown GR, azine dark green BH/C, azine deep black EW, or azine deep black 3RL; a nigrosine compound such as nigrosine, nigrosine salt, or a nigrosine derivative; an acid dye made of a nigrosine compound such as nigrosine BK, nigrosine NB, or nigrosine Z; metal salts of naphthenic acid or higher fatty acid; alkoxyated amine; alkylamide; and quaternary ammonium salt such as benzylmethylhexyldecylammonium or decyltrimethylammonium chloride. Among these positively chargeable charge control agents, the nigrosine compound is particularly preferred for a reason of achieving quicker charge rise characteristic. Two or more types of these positively chargeable charge control agents can be used in combination with each other.

Resin with a quaternary ammonium salt, a carboxylate salt, or a carboxyl group as a functional group may also be used as the positively chargeable charge control agent. More specifically, the following examples can be given: styrene-based resin with a quaternary ammonium salt, acrylic resin with a quaternary ammonium salt, styrene-acrylic resin with a quaternary ammonium salt, polyester resin with a quaternary ammonium salt, styrene-based resin with a carboxylate salt, acrylic resin with a carboxylate salt, styrene-acrylic resin with a carboxylate salt, styrene-based resin with a carboxyl group, acrylic resin with a carboxyl group, styrene-acrylic resin with a carboxyl group, or polyester resin with a carboxyl group. The molecular weight of such resins is not particularly limited but may be an oligomer or a polymer.

For a specific example of the negatively chargeable charge control agent, an organometallic complex or a chelate compound can be given. For the organometallic complex or the chelate compound, it is preferable to use: a metal acetylacetone complex such as aluminum acetylacetone or iron (II) acetylacetone, or a salicylic acid-based metal complex such as 3,5-di-tert-butylsalicylic acid chromium, or salicylic acid-based metal salt. The salicylic acid-based metal complex or the salicylic acid-based metal salt is more preferable. Two or more types of these negatively chargeable charge control agents can be used in combination with each other.

The amount of use of the positively or negatively chargeable charge control agent should preferably be 1.5 parts by mass or more and 15 parts by mass or less, with respect to 100 parts by mass of the total amount of toner, and more preferably be 2.0 parts by mass or more and 8.0 parts by mass or less. If the amount of use of the charge control agent is too

small, it is difficult to stably charge the toner to a predetermined polarity. Thus, there is a case where the image density of the formed image is below a predetermined level or it becomes difficult to maintain the image density for a long time. In addition, in this case, it is difficult to uniformly disperse the charge control agent within the toner, thus making it more likely to cause fogging in the formed image or stain on the latent image bearing member by the toner. On the other hand, if the amount of use of the charge control agent is 10 too large, it is likely to cause insufficient charge of the toner under high temperature and high humidity due to deterioration in environment resistance of the toner. In this case, problems such as image defect in the formed image or stain on the latent image bearing member are more likely to occur.

[Magnetic Powder]

The electrostatic latent image developing toner according to the present disclosure may include magnetic powder as desired. For a preferred example of the magnetic powder, the following can be given: iron such as ferrite or magnetite; ferromagnetic metal such as cobalt or nickel; an alloy including iron and/or ferromagnetic metal; a compound including iron and/or ferromagnetic metal; a ferromagnetic alloy treated by ferromagnetic treatment such as heat treatment; and chromium dioxide.

25 A particle diameter of the magnetic powder should preferably be 0.1  $\mu\text{m}$  or more and 1.0  $\mu\text{m}$  or less, and more preferably be 0.1  $\mu\text{m}$  or more and 0.5  $\mu\text{m}$  or less. In the case of using the magnetic powder having a particle diameter within the range as described above, it is easier to uniformly disperse the 30 magnetic powder within the binder resin.

For the magnetic powder, to improve the dispersibility of the magnetic powder in the binder resin, it is possible to use a magnetic powder that is surface-treated with a surface preparation agent such as a titanium coupling agent or a silane coupling agent.

The amount of use of the magnetic powder, in the case of using the toner as a one component developer, should preferably be 35 parts by mass or more and 60 parts by mass or less, with respect to 100 parts by mass of the total amount of toner, 40 and more preferably be 40 parts by mass or more and 60 parts by mass or less. If the amount of use of the magnetic powder is too large, there is a case where it is difficult to maintain the image density at a desired level for a long time or fixability of the toner onto the paper is extremely reduced. On the other hand, if the amount of use of the magnetic powder is too small, there is a case where the formed image is likely to have fogging or it becomes difficult to maintain the image density at a desired level for a long time. In addition, in the case of using the toner as a two component developer, the amount of 45 50 the magnetic powder should preferably be 20% by mass or less with respect to 100 parts by mass of the total amount of the toner, and more preferably be 15% by mass or less.

[External Additive]

The electrostatic latent image developing toner according 55 to the present disclosure may have a surface treated with an external additive, as desired. It should be noted that in the specification of the present disclosure, toner particles yet to be treated with an external additive are referred to as "toner base particles". The type of the external additive can be selected appropriately from external additives that have been used for toner since before. For specific examples of the preferred external additive, it is possible to give: silica, or metal oxide such as alumina, titanium oxide, magnesium oxide, zinc oxide, strontium titanate, and barium titanate. 60 Two or more types of these external additives can be used in combination with each other. In addition, these external additives can be hydrophobized for use, using a hydrophobizing

agent such as an aminosilane coupling agent or silicone oil. In the case of using a hydrophobized external additive, it becomes easier to suppress decrease in charge amount of the toner under high temperature and high humidity, and also it becomes easier to obtain the toner having excellent fluidity.

A particle diameter of the external additive should preferably be 0.01  $\mu\text{m}$  or more and 1.0  $\mu\text{m}$  or less.

The amount of use of the external additive should preferably be 0.1 parts by mass or more and 10 parts by mass or less, with respect to 100 parts by mass of toner particles before treatment with the external additive (toner base particles), and more preferably be 0.2 parts by mass or more and 5 parts by mass or less.

[Method for Manufacturing the Electrostatic Latent Image Developing Toner]

A method for manufacturing the electrostatic latent image developing toner according to the present disclosure is not particularly limited as long as the method allows mixing of the releasing agent with the binder resin and thereby allows manufacturing of the toner including an optional component as described above as necessary. Preferred methods include a pulverizing method and an aggregation method. In the pulverizing method, essential components such as a binder resin and a releasing agent, and an optional component such as a colorant, a charge control agent, or magnetic powder are mixed. A mixture obtained thereby is melted and kneaded by a melt-kneader such as a single-axis or biaxial extruder, and a product thus obtained from the melting and kneading is pulverized and classified, thereby obtaining toner particles (toner base particles). In the aggregation method, particulates of the components included in the toner, such as the binder resin, the releasing agent, and the colorant, are aggregated in an aqueous medium, thereby obtaining aggregated particles. Next, the aggregated particles are heated so as to coalesce components included in the aggregated particles, thereby obtaining toner particles (toner base particles). Of these methods, the pulverizing method is the more preferable. Generally, an average particle diameter of the toner particles (toner base particles) should preferably be 5  $\mu\text{m}$  or more and 10  $\mu\text{m}$  or less.

The surface of the toner base particles thus obtained may be treated with an external additive as necessary. The method for treating the toner base particles using an external additive is not particularly limited and can be selected appropriately from among known treatment methods using external additives. Specifically, conditions for external addition treatment are adjusted such that the particles of the external additives are not embedded in the toner base particles, and the treatment using the external additive is performed, using a mixer such as a Henschel mixer or a Nauta Mixer.

[Carrier]

The electrostatic latent image developing toner according to the present disclosure can also be mixed with a desired carrier for use as a two component developer. For preparing the two component developer, it is preferable to use a magnetic carrier.

In addition, for an example of a preferred carrier, a carrier having a carrier core coated with resin can be given. For specific examples of the carrier core, it is possible to give: particles of metal such as iron, oxidatively-treated iron, reduced iron, magnetite, copper, silicon steel, ferrite, nickel, or cobalt; particles of an alloy made from these materials and metal such as manganese, zinc, or aluminum; particles of an iron alloy such as a nickel-iron alloy or a cobalt-iron alloy; particles of ceramics such as titanium oxide, aluminum oxide, copper oxide, magnesium oxide, lead oxide, zirconium oxide, silicon carbide, magnesium titanate, barium titanate, lithium

titanate, lead titanate, lead zirconate, or lithium niobate; particles of a high-permittivity substance such as ammonium dihydrogen phosphate, potassium dihydrogen phosphate, or Rochelle salt; and a resin carrier formed by dispersing the above magnetic powder in resin.

For specific examples of the resin for coating the carrier core, it is possible to give: a (meth)acrylic polymer, a styrene-based polymer, a styrene-(meth)acrylic copolymer, an olefin-based polymer (polyethylene, chlorinated polyethylene, or polypropylene), polyvinyl chloride, polyvinyl acetate, polycarbonate, cellulose resin, polyester resin, unsaturated polyester resin, polyamide resin, polyurethane resin, epoxy resin, silicone resin, fluororesin (polytetrafluoroethylene, polychlorotrifluoroethylene, or polyvinylidene fluoride), phenol resin, xylene resin, diallyl phthalate resin, polyacetal resin, or amino resin. Two or more types of these resins can be used in combination with each other.

A particle diameter of the carrier is measured using an electron microscope. The particle diameter of the carrier should preferably be 20  $\mu\text{m}$  or more and 120  $\mu\text{m}$  or less, and more preferably be 25  $\mu\text{m}$  or more and 80  $\mu\text{m}$  or less.

In the case of using the toner according to the present disclosure as a two component developer, a toner content in the two component developer should preferably be 3% by mass or more and 20% by mass or less with respect to the mass of the two component developer, and more preferably be 5% by mass or more and 15% by mass or less. By setting the toner content in the two component developer within such a range, it becomes easier to maintain the image density of the formed image at an appropriate level as well as suppressing toner scatter from the developing device, thus suppressing toner stain on an inner part of the image forming apparatus or toner attachment to transfer paper.

[Thermomechanical Analysis (TMA)]

For the toner according to the present disclosure, the maximum thermal expansion coefficient difference ( $\text{Sw}_{\max} - \text{Sr}_{\max}$ ) that is a difference between the maximum value ( $\text{Sw}_{\max}$ ) of the thermal expansion coefficient of the releasing agent and the maximum value ( $\text{Sr}_{\max}$ ) of the thermal expansion coefficient of the binder resin is 1 or more. It should be noted that the maximum expansion coefficient difference is a difference between the value of  $\text{Sw}_{\max}$  and the value of  $\text{Sr}_{\max}$ , and is a dimensionless value. In addition, the thermal expansion coefficient of the releasing agent reaches the maximum at a temperature of 60°C. or more and 75°C. or less. It should be noted that the maximum value of the thermal expansion coefficient of the releasing agent and the maximum value of the thermal expansion coefficient of the binder resin are measured using a thermomechanical analyzer (TMA). The toner according to the present disclosure includes a combination of the binder resin and the releasing agent having such thermal characteristics, and therefore excels in preservation stability, low temperature fixability, and high temperature offset resistance.

If the maximum thermal expansion coefficient difference ( $\text{Sw}_{\max} - \text{Sr}_{\max}$ ) is too small, at the time of fixing, the releasing agent is difficult to flow out from the toner melted by heating. Therefore, by using the toner of which the maximum thermal expansion coefficient difference ( $\text{Sw}_{\max} - \text{Sr}_{\max}$ ) is too small, it is difficult to obtain sufficient mold releasability, between a heat roller and a toner image. Thus, such toner is poor in low temperature fixability and high temperature offset resistance.

It is possible to adjust the maximum thermal expansion coefficient difference ( $\text{Sw}_{\max} - \text{Sr}_{\max}$ ) by adjusting the maximum value ( $\text{Sw}_{\max}$ ) of the thermal expansion coefficient of the releasing agent and the maximum value ( $\text{Sr}_{\max}$ ) of the thermal expansion coefficient of the binder resin. Then, it is

## 11

possible to adjust the maximum value ( $Sw_{max}$ ) of the thermal expansion coefficient of the releasing agent by adjusting the carbon number distribution of the releasing agent. For example, the maximum value ( $Sw_{max}$ ) of the thermal expansion coefficient of the releasing agent tends to decrease by narrowing the carbon number distribution of the releasing agent, and tends to increase by broadening the carbon number distribution of the releasing agent. The maximum value ( $Sw_{max}$ ) of the thermal expansion coefficient of the releasing agent is not particularly limited as long as the maximum thermal expansion coefficient difference ( $Sw_{max}-Sr_{max}$ ) is 1 or more, but should preferably be 3.0% or more, and more preferably be 3.0% or more and 4.5% or less.

In addition, the maximum value of the thermal expansion coefficient of the binder resin ( $Sr_{max}$ ) is adjustable by, for example, adjusting the molecular weight of the binder resin. The maximum value of the thermal expansion coefficient ( $Sr_{max}$ ) of the binder resin tends to decrease by increasing the molecular weight of the binder resin, and tends to increase by decreasing the molecular weight of the binder resin.

The temperature at which the thermal expansion coefficient of the releasing agent reaches the maximum can be adjusted by adjusting the average carbon number of the releasing agent. For example, it is possible to decrease the temperature at which the thermal expansion coefficient of the releasing agent reaches the maximum by reducing the average carbon number of the releasing agent. In addition, it is possible to increase the temperature at which the thermal expansion coefficient of the releasing agent reaches the maximum by increasing the average carbon number of the releasing agent.

For measurement using the thermomechanical analyzer (TMA), for example, a thermomechanical analyzer ("TMA/SS6100" manufactured by SII Nano Technology) may be used.

The measurement to be performed on the releasing agent and the binder resin by the thermomechanical analyzer (TMA) may be performed on the releasing agent and the binder resin that are materials used for toner preparation, or may be performed on the releasing agent and the binder resin that are separated from the toner. Although the method for separating the releasing agent and the binder resin from the toner is not particularly limited, the following method can be given, for example.

<Method for Separating the Releasing Agent and the Binder Resin>

The toner is immersed in methyl ethyl ketone (MEK), and a sample obtained after allowing the toner to stand for 24 hours at 25° C. is filtered by glass filter (opening standard 11G-3). A filtrate thus obtained is allowed to stand for 12 hours, and a supernatant liquid is taken. The supernatant liquid thus taken is vacuum dried at 60° C., and the binder resin can be obtained as a residue remaining after drying. Next, the residue on the glass filter is immersed in toluene of 50° C., and is allowed to stand for 24 hours at 25° C., thereby

## 12

obtaining a sample. A sample thus obtained is filtered by glass filter (opening standard 11G-3). After allowing a filtrate thus obtained to stand for 12 hours, a supernatant liquid is taken. The supernatant liquid thus taken is vacuum dried at 60° C., and the releasing agent can be obtained as a residue remaining after drying.

As described above, the electrostatic latent image developing toner according to the present disclosure has excellent preservation stability, low temperature fixability, and high temperature offset resistance. Thus, the electrostatic latent image developing toner according to the present disclosure is preferably used in various image forming apparatuses.

## EXAMPLES

15 The following describes the present disclosure in further detail using examples. It should be noted that the present disclosure is not to be limited at all according to the examples.

In Examples and Comparative Examples, releasing agents A to F were used. Methods for manufacturing the releasing agents A to E are described in Preparation Example 1. For the releasing agent F, a commercially available carnauba wax ("Carnauba Wax No. 1 (natural ester wax)" manufactured by TOA KASEI CO., LTD.) was used. Table 1 shows, of ester included in the carnauba wax, the carbon number distribution of the acyl group and the carbon number distribution of the alkyl group derived from alcohol.

## Preparation Example 1

## Preparing Releasing Agents A to E

The releasing agents A to E, which were ester waxes, were prepared according to the following procedures, using a carboxylic acid component and an alcohol component that have a carbon number distribution as described in Table 1.

A four neck flask of a 1 liter capacity, having a thermometer, a nitrogen introduction tube, a stirrer ("Homogenizer (Ultra-Turrax T 50)" manufactured by Ika Works), and a cooling tube, was used as a reaction container. To the reaction container, 50 parts by mass of a carboxylic acid component of the type described in Table 2 and 50 parts by mass of an alcohol component of the type described in Table 2, were added. Next, under nitrogen gas stream, by causing a reaction under normal pressure at 220° C. and an agitating speed of 3000 rpm for 15 hours while distilling away by-product water, an esterification crude product was obtained. 20 parts by mass of ion-exchange water was added to 100 parts by mass of the esterification crude product thus obtained, which was stirred at an agitation speed of 3500 rpm at 70° C. for 30 minutes, and then was allowed to stand for 30 minutes, and an aqueous layer was separated and removed. Water washing was repeatedly performed until pH of the separated aqueous layer became neutral. The remaining ester layer was heated to 180° C. under a condition of reduced pressure of 1 kPa so as to remove volatile, thereby obtaining ester wax.

TABLE 1

| Synthetic ester wax | Carboxylic component | Behenic acid A (% by mass) | Carbon number |    |    |    |    |    |    |    |    |    |
|---------------------|----------------------|----------------------------|---------------|----|----|----|----|----|----|----|----|----|
|                     |                      |                            | 12            | 14 | 16 | 18 | 20 | 22 | 24 | 26 | 28 | 30 |
|                     |                      | Behenic acid B (% by mass) | —             | —  | —  | 6  | 14 | 80 | —  | —  | —  | —  |
|                     |                      | Palmitic acid (% by mass)  | —             | 1  | 95 | 4  | —  | —  | —  | —  | —  | —  |

TABLE 1-continued

|                   |  | Carbon number                                   |    |    |    |    |    |    |    |    |    |    |    |    |
|-------------------|--|-------------------------------------------------|----|----|----|----|----|----|----|----|----|----|----|----|
|                   |  | 12                                              | 14 | 16 | 18 | 20 | 22 | 24 | 26 | 28 | 30 | 32 | 34 | 36 |
| Alcohol component |  | Behenyl alcohol A<br>(% by mass)                | —  | —  | —  | 2  | 6  | 85 | 7  | —  | —  | —  | —  | —  |
|                   |  | Behenyl alcohol B<br>(% by mass)                | —  | —  | —  | 8  | 16 | 70 | 6  | —  | —  | —  | —  | —  |
|                   |  | Stearyl alcohol A<br>(% by mass)                | —  | —  | 2  | 96 | 2  | —  | —  | —  | —  | —  | —  | —  |
|                   |  | Stearyl alcohol B<br>(% by mass)                | —  | —  | 16 | 80 | 4  | —  | —  | —  | —  | —  | —  | —  |
|                   |  | Acyl group<br>(% by mass)                       | 3  | 6  | 13 | 12 | 28 | 13 | 18 | 4  | 3  | —  | —  | —  |
|                   |  | Alkyl group derived from alcohol<br>(% by mass) | —  | —  | —  | —  | —  | 2  | 3  | 2  | 5  | 13 | 54 | 18 |
| Carnauba wax      |  |                                                 |    |    |    |    |    |    |    |    |    |    |    | 3  |

TABLE 2

| Releasing agent | Carboxylic component type | Alcohol component type |
|-----------------|---------------------------|------------------------|
| A               | Behenic acid B            | Stearyl alcohol A      |
| B               | Behenic acid A            | Stearyl alcohol B      |
| C               | Palmitic acid             | Behenyl alcohol B      |
| D               | Behenic acid A            | Behenyl alcohol B      |
| E               | Behenic acid A            | Behenyl alcohol A      |

## Examples 1 and 2, and Comparative Examples 1 to 4

48 parts by mass of polyester resin A and 39 parts by mass of polyester resin B as described below, as the binder resin, 8 parts by mass of the colorant (“Carbon Black (MA-100)” manufactured by Mitsubishi Chemical Corporation), 2 parts by mass of the charge control agent (“N-01” manufactured by ORIENT CHEMICAL INDUSTRIES, CO., Ltd.), and 3 parts by mass of the releasing agent of the types described in Table 2 were mixed using a Henschel mixer (“FM-10” manufactured by Mitsui Mining Company, Ltd.). The mixture thus obtained was melted and kneaded using a biaxial extruder (“TEM-26SS” manufactured by Toshiba Machine Co. Ltd.), thereby obtaining a product resulting from the melting and kneading. The product resulting from the melting and kneading, after being cooled, was coarsely pulverized down to an average particle diameter of approximately 2 mm, using a Rotoplex grinder (manufactured by TOA MACHINERY MFG. GO., LTD.). Next, using a turbo mill (“RS type” manufactured by TURBO KOGYO CO., Ltd.), the coarsely pulverized product was finely pulverized. The finely pulverized product was classified using an air classifier (“EJ-L-3 (LABO type)” manufactured by Nittetsu Mining Co., Ltd.), thereby obtaining toner base particles having a volume average particle diameter of 7.0  $\mu\text{m}$ . The volume average particle diameter of the toner base particles thus obtained was measured using a particle size distribution measurement device (“Multisizer 3” manufactured by Beckman Coulter, Inc.).

Polyester resin A: Mass average molecular weight (Mw) 320000, Glass transition point (Tg) 66°C.

Polyester resin B: Mass average molecular weight (Mw) 80000, Glass transition point (Tg) 62°C.

To 100 parts by mass of the toner base particles thus obtained, 1.5 parts by mass of positively-chargeable silica particulates (“RA 200” manufactured by NipponAerosil Co., Ltd.) and 1.0 parts by mass of titanium oxide (“MT-500B” manufactured by TAYCA CORPORATION) were added.

These were mixed at a rotation rate of 3500 rpm for 5 minutes using a Henschel mixer (“FM-10” manufactured by Mitsui Mining Company, Ltd.) for performing the external addition treatment, thereby obtaining the toner as described in each of Examples 1 and 2 and Comparative Examples 1 to 4.

## [Thermomechanical Analysis (TMA)]

The binder resin and the releasing agent were separated from the toner in each of Examples 1 and 2 and Comparative Examples 1 to 4, according to the method below. Next, with the binder resin and the releasing agent that are obtained by the separation, the thermal expansion coefficient curve of the binder resin and the thermal expansion coefficient curve of the releasing agent were measured according to a TMA measurement method as described below. Next, the maximum thermal expansion coefficient ( $\text{Sr}_{\max}$ ) of the binder resin, the maximum thermal expansion coefficient ( $\text{Sw}_{\max}$ ) of the releasing agent, and the temperature at which the thermal expansion coefficient of the releasing agent reached the maximum were obtained from the obtained thermal expansion coefficient curves of the binder resin and the releasing agent. The maximum thermal expansion coefficient difference ( $\text{Sw}_{\max} - \text{Sr}_{\max}$ ) was calculated from the maximum thermal expansion coefficient ( $\text{Sw}_{\max}$ ) of the releasing agent and the maximum thermal expansion coefficient ( $\text{Sr}_{\max}$ ) of the binder resin. Table 3 shows a result of the measurement, regarding the toner in each of Examples 1 and 2 and Comparative Examples 1 to 4, of the maximum thermal expansion coefficient ( $\text{Sr}_{\max}$ ) of the binder resin, the maximum thermal expansion coefficient ( $\text{Sw}_{\max}$ ) of the releasing agent, the temperature at which the thermal expansion coefficient of the releasing agent reaches the maximum, and the maximum thermal expansion coefficient difference ( $\text{Sw}_{\max} - \text{Sr}_{\max}$ ). In addition, FIG. 1 shows the thermal expansion coefficient curves of the releasing agent and the binder resin that are included in the toner in Example 1. In addition, FIGS. 2 to 6 show the thermal expansion coefficient curves of the releasing agent and the binder resin that are included in the toner in each of Example 2 and Comparative Examples 1 to 4.

## &lt;Method for Separating the Releasing Agent and the Binder Resin&gt;

10 g of toner was immersed in 200 ml of methyl ethyl ketone (MEK), which was allowed to stand at 25°C. for 24 hours, thereby obtaining a sample. Then, the sample thus obtained was filtered by glass filter (opening standard 11G-3). A filtrate was allowed to stand for 12 hours, and a supernatant liquid was taken. The supernatant liquid thus taken was vacuum dried at 60°C., thereby obtaining the binder resin as a residue remaining after drying. Next, the residue on the

glass filter was immersed in 300 ml of toluene of 50° C., which was allowed to stand at 30° C. for 24 hours, and a sample was obtained. The sample thus obtained was filtered by glass filter (opening standard 11 G-3). After allowing the filtrate to stand for 12 hours, the supernatant liquid was taken. The supernatant liquid was vacuum dried at 60° C., thereby obtaining the releasing agent as a residue after drying.

## &lt;TMA Measurement Method&gt;

For the thermomechanical (TMA) measurement, the measurement was performed using a thermomechanical analyzer ("TMA/SS6100" manufactured by SII Nano Technology). The linear expansion coefficient was obtained using a measurement method according to the "Testing method for linear thermal expansion coefficient of plastics by thermomechanical analysis" by JIS K 7197. The measurement was performed by varying the measurement temperature from 25° C. to 160° C. at a rate of temperature increase of 2.0° C./minute. 0.3 g of the sample was shaped to a diameter of 1 cm and a thickness of 2 mm. The measurement was performed by setting device conditions to: probe diameter of 1.0 mm; probe diameter of 2.0 mm, probe load of 50 mN, and nitrogen flow at 80 ml/minute. It should be noted that the thermal expansion coefficient and the linear expansion coefficient have the same meaning.

FIG. 1 shows the thermal expansion coefficient curve of each of the releasing agent and the binder resin that are included in the toner in Example 1. From the thermal expansion coefficient curve shown in FIG. 1, the maximum thermal expansion coefficient ( $S_{r_{max}}$ ) of the binder resin and the maximum thermal expansion coefficient ( $S_{w_{max}}$ ) of the releasing agent were obtained as described in Table 3. In addition, from the thermal expansion coefficient curve of the releasing agent, the temperature at which the thermal expansion coefficient reached the maximum was obtained as described in Table 3.

FIGS. 2 to 6 show the thermal expansion coefficient curve of each of the releasing agent and the binder resin that are included in the toner in each of Example 2 and Comparative Examples 1 to 4. From each of the thermal expansion coefficient curves shown in FIGS. 2 to 6, the maximum thermal expansion coefficient ( $S_{r_{max}}$ ) of the binder resin and the maximum thermal expansion coefficient ( $S_{w_{max}}$ ) of the releasing agent were obtained as described in Table 3. In addition, from the thermal expansion coefficient curve of the releasing agent, the temperature at which the thermal expansion coefficient reached the maximum was obtained as described in Table 3. It should be noted that the thermal expansion coefficient curve of the binder resin included in the toner in each of Example 2 and Comparative Examples 1 to 4 was the same as the thermal expansion coefficient curve of the binder resin included in the toner in Example 1.

## &lt;&lt;Evaluation 1&gt;&gt;

Regarding the toner in each of Examples 1 and 2 and Comparative Examples 1 to 4, the heat-resisting preservation stability and the dispersibility of the releasing agent were evaluated according to the method below. Table 3 shows a result of the evaluation of the heat-resisting preservation stability of the toner and the dispersibility of the releasing agent in the toner in each of Examples 1 and 2 and Comparative Examples 1 to 4.

## &lt;Evaluation Method for Heat-Resisting Preservation Stability&gt;

10 g of toner was weighed in a sample bottle made of glass, and the sample bottle containing the toner, which was not sealed with a stopper, was allowed to stand for 100 hours in a constant temperature reservoir ("CONVECTION OVEN" manufactured by SANYO Electric Co., Ltd.) of 50° C. Next, a sieve of 26 mesh having a known mass was attached to a powder tester ("TYPE PT-E 84810" manufactured by Hosokawa Micron Corporation), and the toner after standing at high temperature was placed on the sieve and weighed

before sieving. Next, the toner was sieved for 20 seconds on a condition of rheostat 2.5. Next, the mass of the residual toner remaining on the sieve was measured. The heat-resisting preservation stability was evaluated according to a reference as below.

Good: Residual toner on the mesh was 0.2 g or less.

Poor: Residual toner on the mesh was over 0.2 g.

## &lt;Evaluation Method for Dispersibility of the Releasing Agent&gt;

5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035

portion was present inside, and a crease was frictioned back and forth 5 times with a weight of 1 kg having a bottom covered with a cloth. After the friction, the paper was unfolded, to determine that the result was passing if the peeling of the toner was 1 mm or less and that the result was failed if the peeling of the toner was over 1 mm. The fixing temperature was evaluated by increasing the temperature from

est temperature at which the offset did not occur as a high temperature offset non-occurrence temperature.

Good: The high temperature offset non-occurrence temperature was 200° C. or more.

Poor: The high temperature offset non-occurrence temperature was below 200° C.

TABLE 3

|                                                                                  | Examples |      | Comparative Examples |      |      |         |
|----------------------------------------------------------------------------------|----------|------|----------------------|------|------|---------|
|                                                                                  | 1        | 2    | 1                    | 2    | 3    | 4       |
| Type of releasing agent                                                          | A        | B    | C                    | D    | E    | F       |
| Maximum thermal expansion coefficient of binder resin ( $S_{r_{max}}$ ) [%]      | 0.60     | 0.60 | 0.60                 | 0.60 | 0.60 | 0.60    |
| Maximum thermal expansion coefficient of releasing agent ( $S_{w_{max}}$ ) [%]   | 3.00     | 4.20 | 2.30                 | 1.58 | 2.66 | 1.10    |
| Thermal expansion peak temperature of releasing agent [° C.]                     | 63       | 70   | 57                   | 71   | 80   | 75      |
| Maximum thermal expansion coefficient difference ( $S_{w_{max}} - S_{r_{max}}$ ) | 2.40     | 3.60 | 1.70                 | 0.98 | 2.06 | 0.50    |
| Evaluation 1                                                                     |          |      |                      |      |      |         |
| Dispersibility of releasing agent                                                | Good     | Good | Good                 | Good | Good | Average |
| Heat-resisting preservation stability                                            |          |      |                      |      |      |         |
| Residual toner on mesh [g]                                                       | 0.20     | 0.18 | 0.30                 | 0.17 | 0.13 | 0.15    |
| Evaluation                                                                       | Good     | Good | Poor                 | Good | Good | Good    |
| Evaluation 2                                                                     |          |      |                      |      |      |         |
| Low temperature fixability                                                       |          |      |                      |      |      |         |
| Lowest fixing temperature [° C.]                                                 | 155      | 160  | 155                  | 170  | 175  | 165     |
| Evaluation                                                                       | Good     | Good | Good                 | Poor | Poor | Poor    |
| High temperature offset resistance                                               |          |      |                      |      |      |         |
| High temperature offset non-occurrence temperature [° C.]                        | 200      | 210  | 190                  | 190  | 210  | 195     |
| Evaluation                                                                       | Good     | Good | Poor                 | Poor | Good | Poor    |

140° C. in increments of 5° C., and the low temperature fixability was evaluated according to an evaluation reference below, assuming a lowest fixing temperature at which the peeling of the toner was determined to be pass as the lowest fixing temperature.

Good: The lowest fixing temperature was 160° C. or less.

Poor: The lowest fixing temperature was over 160° C.

<Evaluation Method for High Temperature Offset Resistance>

The same developing device and toner container that were used in the measurement according to the evaluation method for low temperature fixability were used. Using the evaluation device, a toner image of 2 cm×3 cm (patch sample) was output onto the recording medium as an unfixed image such that the toner mount amount was 1.8 mg/cm<sup>2</sup>. Next, using the fixability tester, the unfixed image of the patch sample was fixed at a linear speed of 280 mm/second. Using the fixed image, whether or not a high temperature offset occurred was visually checked. The evaluation was performed by increasing the fixing temperature from 140° C. in increments of 5° C., and the high temperature offset resistance was evaluated according to an evaluation reference below, assuming a high-

est temperature at which the offset did not occur as a high temperature offset non-occurrence temperature.

Good: The high temperature offset non-occurrence temperature was 200° C. or more.

Poor: The high temperature offset non-occurrence temperature was below 200° C.

For the electrostatic latent image developing toner in each of Examples 1 and 2, the maximum thermal expansion coefficient difference ( $S_{w_{max}} - S_{r_{max}}$ ) that is a difference between the maximum value of the thermal expansion coefficient ( $S_{w_{max}}$ ) of the releasing agent and the maximum value of the thermal expansion coefficient ( $S_{r_{max}}$ ) of the binder resin is 1 or more, and the temperature at which the thermal expansion coefficient in the thermal expansion coefficient curve of the releasing agent reaches the maximum is 60° C. or more and 75° C. or less. It is shown that such electrostatic latent image developing toner has excellent preservation stability, low temperature fixability, and high temperature offset resistance.

For the electrostatic latent image developing toner in Comparative Example 1, the temperature at which the thermal expansion coefficient of the releasing agent reaches the maximum was too low. In this case, it is shown that it is difficult to obtain the toner having excellent preservation stability and high temperature offset resistance.

For the electrostatic latent image developing toner in each of Comparative Examples 2 and 4, the thermal expansion coefficient difference ( $S_{w_{max}} - S_{r_{max}}$ ) was too small. In this case, it is shown that it is difficult to obtain the toner having

**19**

excellent low temperature fixability and high temperature offset resistance. In addition, it is shown that for the toner in Comparative Example 4, the wax is difficult to sufficiently disperse within the toner.

According to the electrostatic latent image developing toner in Comparative Example 3, it is shown that: if the temperature at which the thermal expansion coefficient of the releasing agent reaches the maximum is too high, it is difficult to obtain the toner having excellent low temperature fixability.

What is claimed is:

**1. An electrostatic latent image developing toner comprising**

at least a binder resin and a releasing agent, wherein the releasing agent includes an ester wax from carboxylic acid component A and alcohol component B or an ester wax from carboxylic acid component B and alcohol component A,

the carboxylic acid component A includes a portion having carbon number 18 of a mass fraction 0.01, a portion having carbon number 20 of a mass fraction 0.10, a portion having carbon number 22 of a mass fraction 0.87, and a portion having carbon number 24 of a mass fraction 0.02,

the carboxylic acid component B includes a portion having carbon number 18 of a mass fraction 0.06, a portion having carbon number 20 of a mass fraction 0.14, and a portion having carbon number 22 of a mass fraction 0.80,

the alcohol component A includes a portion having carbon number 16 of a mass fraction 0.02, a portion having carbon number 18 of a mass fraction 0.96, and a portion having carbon number 20 of a mass fraction 0.02,

10  
20  
30

**20**

the alcohol component B includes a portion having carbon number 16 of a mass fraction 0.16, a portion having carbon number 18 of a mass fraction 0.80, and a portion having carbon number 20 of a mass fraction 0.04,

a maximum thermal expansion coefficient difference ( $Sw_{max} - Sr_{max}$ ) is 1 or more, the maximum thermal expansion coefficient being a difference between a maximum value ( $Sw_{max}$ ) of a thermal expansion coefficient of the releasing agent and a maximum value ( $Sr_{max}$ ) of a thermal expansion coefficient of the binder resin that are measured using thermomechanical analysis (TMA),

a temperature at which the thermal expansion coefficient of the releasing agent reaches a maximum is 60° C. or more and 75° C. or less,

the releasing agent has an average carbon number of 39 or more and 41 or less, and

an amount of the releasing agent is 1 part by mass or more and 5 parts by mass or less, with respect to 100 parts by mass of the binder resin.

**2. An electrostatic latent image developing toner according to claim 1, wherein**

the releasing agent is a synthetic ester wax.

**3. An electrostatic latent image developing toner according to claim 1, wherein**

the maximum value ( $Sw_{max}$ ) of the thermal expansion coefficient of the releasing agent is 3.0% or more.

**4. An electrostatic latent image developing toner according to claim 1, wherein**

the electrostatic latent image developing toner is pulverized toner.

\* \* \* \* \*